



US011015271B2

(12) **United States Patent**  
**Lawrence**

(10) **Patent No.:** **US 11,015,271 B2**  
(45) **Date of Patent:** **May 25, 2021**

(54) **WET-ACTIVATED COOLING FABRIC**

(71) Applicant: **MPUSA, LLC**, Brentwood, NH (US)

(72) Inventor: **David Chad Lawrence**, Alpharetta, GA (US)

(73) Assignee: **MPUSA, LLC**, Brentwood, NH (US)

(\*) Notice: Subject to any disclaimer, the term of this patent is extended or adjusted under 35 U.S.C. 154(b) by 259 days.

(21) Appl. No.: **16/100,939**

(22) Filed: **Aug. 10, 2018**

(65) **Prior Publication Data**

US 2018/0347084 A1 Dec. 6, 2018

**Related U.S. Application Data**

(63) Continuation of application No. PCT/US2017/035734, filed on Jun. 2, 2017.  
(Continued)

(51) **Int. Cl.**  
*D04B 21/08* (2006.01)  
*D04B 1/16* (2006.01)  
*D04B 21/16* (2006.01)  
*D02G 3/04* (2006.01)  
*D02G 3/36* (2006.01)  
(Continued)

(52) **U.S. Cl.**  
CPC ..... *D04B 21/08* (2013.01); *D02G 3/045* (2013.01); *D02G 3/36* (2013.01); *D02G 3/38* (2013.01); *D04B 1/16* (2013.01); *D04B 21/16* (2013.01); *D04B 21/18* (2013.01); *D10B 2331/02* (2013.01); *D10B 2331/04* (2013.01); *D10B 2331/10* (2013.01); *D10B 2401/02* (2013.01); *D10B 2401/061* (2013.01); *D10B*

2403/02 (2013.01); *D10B 2403/021* (2013.01); *D10B 2501/00* (2013.01)

(58) **Field of Classification Search**

CPC ..... D04B 21/06; D04B 21/08; D04B 21/16; D04B 21/18; D04B 23/22  
See application file for complete search history.

(56) **References Cited**

**U.S. PATENT DOCUMENTS**

3,922,888 A 12/1975 Patterson  
3,952,555 A 4/1976 Lesley  
(Continued)

**FOREIGN PATENT DOCUMENTS**

JP 11984004789 U 1/1984  
JP 3174889 U 4/2012  
(Continued)

**OTHER PUBLICATIONS**

International Search Report and Written Opinion dated Nov. 27, 2017, from International Application No. PCT/US2017/035734, 16 sheets.

(Continued)

*Primary Examiner* — Danny Worrell

(74) *Attorney, Agent, or Firm* — Carter DeLuca & Farrell LLP

(57) **ABSTRACT**

Disclosed herein is a knitted multi-layer fabric construction that provides the ability to cool skin to below a current temperature whether wetted or dry. The knit uses four separate yarns which collectively work together to produce enhanced cooling. Knits can include warp knit, seamless, hosiery, flat bed, spacer, and double knits. Various finishing methods may also be employed to enhance the cooling power of the fabric.

**20 Claims, 9 Drawing Sheets**



## Related U.S. Application Data

(60) Provisional application No. 62/345,321, filed on Jun. 3, 2016.

## (51) Int. Cl.

D02G 3/38 (2006.01)  
D04B 21/18 (2006.01)

## (56) References Cited

## U.S. PATENT DOCUMENTS

|                |         |                        |               |  |
|----------------|---------|------------------------|---------------|--|
| 4,530,873 A *  | 7/1985  | Okada .....            | B32B 5/026    |  |
|                |         |                        | 442/79        |  |
| 4,638,648 A    | 1/1987  | Gajjar                 |               |  |
| 4,688,403 A    | 8/1987  | Gajjar                 |               |  |
| 5,029,457 A    | 7/1991  | Gajjar                 |               |  |
| 5,065,600 A *  | 11/1991 | Byles .....            | A61F 13/15577 |  |
|                |         |                        | 66/193        |  |
| 5,217,782 A    | 6/1993  | Moretz et al.          |               |  |
| 5,312,667 A *  | 5/1994  | Lumb .....             | D04B 21/207   |  |
|                |         |                        | 428/91        |  |
| 5,596,888 A *  | 1/1997  | McLarty, III et al.    |               |  |
| 5,735,145 A *  | 4/1998  | Pernick .....          | A61F 13/53    |  |
|                |         |                        | 66/196        |  |
| 5,899,095 A    | 5/1999  | Spillane               |               |  |
| 6,151,928 A *  | 11/2000 | Anyon .....            | D04B 1/16     |  |
|                |         |                        | 66/196        |  |
| 6,745,601 B2   | 6/2004  | Pierelli               |               |  |
| 6,770,581 B1   | 8/2004  | DeMott et al.          |               |  |
| 6,986,270 B2 * | 1/2006  | Miller, III .....      | D04B 1/14     |  |
|                |         |                        | 66/202        |  |
| 7,360,378 B2 * | 4/2008  | Foshee .....           | D04B 1/14     |  |
|                |         |                        | 66/196        |  |
| 7,465,683 B2   | 12/2008 | McMurray               |               |  |
| 8,088,698 B2 * | 1/2012  | Polegato Moretti ..... | A41D 31/125   |  |
|                |         |                        | 442/414       |  |

|                   |         |                        |              |  |
|-------------------|---------|------------------------|--------------|--|
| 8,334,134 B2 *    | 12/2012 | Young .....            | A61B 10/0045 |  |
|                   |         |                        | 435/309.1    |  |
| 9,506,187 B2      | 11/2016 | Minko et al.           |              |  |
| 9,725,835 B2 *    | 8/2017  | Vaglio Tessitore ..... | D04B 1/16    |  |
| 9,828,705 B1 *    | 11/2017 | Shiue .....            | D04B 1/12    |  |
| 10,428,448 B2 *   | 10/2019 | Lawrence .....         | D02G 3/045   |  |
| 10,584,432 B2 *   | 3/2020  | Akita .....            | D04B 1/12    |  |
| 2003/0051512 A1   | 3/2003  | Pierelli               |              |  |
| 2007/0163305 A1   | 7/2007  | Baer et al.            |              |  |
| 2008/0072629 A1   | 3/2008  | Gehring                |              |  |
| 2011/0262951 A1 * | 10/2011 | Young .....            | G01N 1/04    |  |
|                   |         |                        | 435/29       |  |
| 2012/0177904 A1 * | 7/2012  | Gehring, Jr. .....     | D04B 21/10   |  |
|                   |         |                        | 428/220      |  |

## FOREIGN PATENT DOCUMENTS

|    |               |         |  |
|----|---------------|---------|--|
| JP | 2013249560 A  | 12/2013 |  |
| JP | 2014141759 A  | 8/2014  |  |
| KR | 10-0403199 B1 | 10/2003 |  |
| KR | 1020020060878 | 10/2003 |  |
| KR | 10-1556411 B1 | 9/2015  |  |

## OTHER PUBLICATIONS

International Written Opinion of International Preliminary Examining Authority dated Jul. 23, 2018, from International Application No. PCT/US2017/035734, 9 sheets.

Notification of Reasons for Refusal dated Mar. 3, 2020 for Japanese Patent Application No. 2018-562524.

Office Action dated Jun. 12, 2019, from corresponding U.S. Appl. No. 16/077,353, 12 sheets.

\* cited by examiner



FIG. 1



FIG. 2A



FIG. 2B



FIG. 2C



FIG. 2D



FIG. 3A



FIG. 3B



FIG. 3C



FIG. 3D



FIG. 3E



FIG. 4



FIG. 5



FIG. 6



FIG. 7A



FIG. 7B



FIG. 7C



FIG. 7D



FIG. 8



SEAMLESS KNIT FACE

FIG. 9A



SEAMLESS KNIT BACK

FIG. 9B

**1**  
**WET-ACTIVATED COOLING FABRIC**

**CROSS-REFERENCE TO RELATED  
APPLICATION**

The present application is a continuation application of International Application No.: PCT/US2017/035734, filed Jun. 2, 2017, the entire contents of which are hereby incorporated by reference in their entirety, and which claims priority to U.S. Provisional Patent Application Ser. No. 62/345,321, filed Jun. 3, 2016, the entire contents of which are hereby incorporated by reference in their entirety.

**BACKGROUND**

(1) Field of Invention

The present invention relates generally to textile fabrics and, more particularly, to multi-layer knitted fabric constructions that provide the ability to cool skin below a current temperature of the skin for a longer duration primarily when wetted but secondarily in a dry state.

(2) Description of Prior Art

Previous wet-activated cooling fabrics have used woven and double knit constructions using absorbent yarns which have moisture absorbing properties. A first layer, located next to the skin, provides a sustained cooling effect. However, such fabrics generally quickly dry out and/or warm up to the skin temperature of the user, negating any cooling effect. Therefore, a need exists for a multi-layer cooling fabric employing more advanced yarns and construction techniques which can provide a sustained cooling effect for a greater amount of time.

**SUMMARY OF THE INVENTION**

The present invention relates generally to textile fabrics and, more particularly, to multi-layer knitted fabric constructions that provide the ability to cool skin below a current temperature of the skin for a longer duration, primarily when wetted, but secondarily in a dry state.

**BRIEF DESCRIPTION OF THE DRAWINGS**

FIG. 1 depicts a representational cross-sectional view of the cooling fabric showing the different layers of the fabric.

FIGS. 2A-2D depict cross sectional views of yarn filaments used in construction of the cooling fabric.

FIGS. 3A-3E depict a pattern for making a warp knit construction, showing the placement of each yarn in the cooling fabric.

FIG. 4 depicts a brushing process.

FIG. 5 depicts an embossing process.

FIG. 6 depicts an image of a brushed and embossed cooling fabric.

FIGS. 7A-7D depict yarns for use in seamless knitting constructions.

FIG. 8 depicts the yarns of FIGS. 7A-7D used in a seamless knit construction.

FIGS. 9A and 9B depicts faces and backs, respectively, of a seamless knit cooling fabric.

**2**

**DETAILED DESCRIPTION**

**Warp Knit Construction**

As shown in FIG. 1, an embodiment of the cooling fabric 100 is intended to be worn next to the skin 102 of a user, such as an athlete. The cooling fabric 100 may form an entire garment, such as a shirt or a pair of shorts, or be strategically integrated into garments where extra cooling is needed, such as near the shoulders/underarms of a user. The cooling fabric 100 may also be utilized to form standalone cooling products such as headbands, towels, hats, etc.

The layers of cooling fabric 100 depicted in FIG. 1 in cross-section are shown separated for clarity and illustrative purposes. In the actual manufactured fabric, the different layers 104-108 are interconnected in a knit construction that is described with reference to FIGS. 3A-3E, for example.

A first layer 104 of the cooling fabric 100, to be worn against the skin 102, is preferably formed of a combination of a stretchable synthetic yarn and an evaporative yarn. Suitable stretchable synthetic yarns include, but are not limited to, spandex, lycra or elastane. Preferably, spandex is used in the construction of cooling fabric 100. A cross-section of a single filament of a stretchable synthetic yarn, such as spandex, is depicted in FIG. 2D. However, the spandex may be omitted from first layer 104 if stretch or draping qualities are not needed for cooling fabric 100.

The evaporative yarn of first layer 104, together with the spandex, creates hydrophobic & hydrophilic channels for perspiration to enter the absorbent center of cooling fabric 100 while also allowing the chilled (e.g., 60° F.) center to provide conductive cooling against skin 102 (e.g., at an average skin temperature of 93.2° F.) as shown by the arrows near skin 102. The evaporative yarn of first layer 104 is preferably a nylon or polyester yarn having a unique cross-section (as seen in FIG. 2A) and is embedded with minerals (e.g., jade or mica) to transport and evaporate moisture from skin 102 while still providing conductive cooling from center layer 106 while also a cooling touch from layer 104. Examples of suitable evaporative yarns include AQUA-X and ASKIN, both manufactured by Hyosung Corporation of the Republic of Korea, both of which also provide UV protection.

The second layer 106 of cooling fabric 100 is formed from a highly absorbent yarn designed to absorb and hold moisture that is wicked from skin 102 by first layer 104. The high absorbance of the second layer 106 is also important to provide a cooling effect to skin 102. That is, because the second layer 106 is highly absorbent, it is able to retain a greater quantity of cooled water when wetted while still providing the ability to absorb wicked moisture.

Second layer 106 is preferably formed from a conjugated bi-component polyester and nylon yarn with a special star-shaped cross-section (the star-shaped cross-section is formed as the result of a treatment applied after cooling fabric 100 is knitted) as depicted in FIG. 2B. Such a yarn is more absorbent than traditional absorbent yarns used in most cooling fabrics. An example of a yarn suitable for use in the second layer 106 is Hyosung MIPAN XF. The yarn utilized in the second layer 106 is preferably Hyosung MIPAN XF which has a wicking rate and a wicking distance more than twice that of cotton of equivalent density.

The third layer 108 of cooling fabric 100 is formed from a yarn designed to transport moisture and provide a cool touch. The third layer 108 allows the moisture trapped in second layer 106 to evaporate into the ambient air and also allows ambient air to move into second layer 106 to cool the center of cooling fabric 100. A cross-section of a single filament of a yarn suitable for use in third layer 108 is depicted in FIG. 2C.

The cooling effect for cooling fabric 100 follows the principles of evaporative cooling. This principle details that water must have heat applied to change from a liquid to a vapor. Once evaporation occurs, this heat from the liquid water is taken due to evaporation resulting in cooler liquid. Once the cooling fabric 100 is wetted with water and preferably wringed to remove excess water, snapping or twirling in the air is a recommended process as it helps facilitate and expedite the moisture movement from the second layer 106, where water is stored, to the outer evaporative layers 104 and 108, where water evaporation occurs. Snapping or twirling in the air also increases the evaporation rate and decreases the material temperature more rapidly by exposing more surface area of the material to air and increased air flow. More specifically, the cooling fabric 100 functions as a device that facilitates and expedites the evaporative process.

Once the temperature of the remaining water in the outer evaporative layer 108 drops through evaporation, a heat exchange happens within water through convection, between water and fabric through conduction, and within fabric through conduction. Thus, the temperature of cooling fabric 100 drops. The evaporation process further continues by wicking water away from the layer 106 to layers 104 and 108 until the stored water is used up. The evaporation rate decreases as the temperature of cooling fabric 100 drops. The temperature of cooling fabric 100 drops gradually to a certain point where equilibrium is reached between the rate of heat absorption into material from environment and heat release by evaporation.

Once the wetted cooling fabric 100 is placed onto one's skin, cooling energy from the cooling fabric 100 is transferred through conduction. After the cooling energy transfer has occurred, the temperature of the cooling fabric increases to equilibrate with the skin temperature. Once this occurs, the wetted cooling fabric 100 can easily be re-activated by the snapping or the twirling method to again drop the temperature.

The various views depicted in FIGS. 2A-2D are cross-sectional diagrams of a single filament used in the different yarns for layers 104-108. However, each yarn used in the present invention contains multiple filaments.

The four-yarn combination utilized in cooling fabric 100 allows for more absorption of water to occur while transporting water efficiently through cooling fabric 100 to create an evaporative cooling effect which increases the conductive cooling effect of cooling fabric 100. Further benefits of cooling fabric 100 include:

Cool touch provided by third layer 108 (exterior) and first layer 104 (against skin 102) when the cooling fabric 100 is dry. A cool touch fabric is a fabric that physically feels cooler than the ambient air when touched by a user, whether wet or dry.

Temperature decrease of the fabric surface by up to 30° F. below average body temperature (e.g., at 98.6° F.) when wet and activated through wringing, snapping or twirling.

Up to a 30% increase in conductive cooling power measured in Watts/m<sup>2</sup> when compared to other fabrics such as cotton.

Cooling for up to two hours after wetting depending on ambient air conditions.

UV protection.

Next, with reference to FIGS. 3A-3E, the unique knitting construction of cooling fabric 100 is described which allows for four different yarns to be used in the same material. Preferably, a warp knit is used during the construction of

cooling fabric 100. Warp knits include, but are not limited to, tricot, raschel, spacer, and lace.

Examples of warp knit tricot 4-bar will be described herein. A first example for warp knit tricot 4-bar construction, depicted in FIGS. 3A-3E, utilizes the following stitch and yarn combinations:

FIG. 3A—Bar 1-1-0/2-3 (evaporative yarn such as AQUA X)

FIG. 3B—Bar 2-1-2/1-0 (absorbent yarn such as MIPAN XF)

FIG. 3C—Bar 3-0-1/2-1 (evaporative yarn such as ASKIN)

FIG. 3D—Bar 4-1-0/1-2 (elastic yarn such as Spandex). Preferably, bar 1 is a 35 Denier/24 filament nylon fully drawn yarn; bar 2 is a 50 Denier/48 filament conjugated polyester/nylon bi-component fully drawn yarn; bar 3 is a 75 Denier/36 filament polyester draw textured yarn; and bar 4 is a 40 Denier spandex. This configuration results in a fabric having a density of 100-600 g/m<sup>2</sup>, but more preferably 160-400 g/m<sup>2</sup>. The combined multi-layer cooling fabric 100 resulting from this stitch is depicted in FIG. 3E.

The yarn Deniers and filament counts used on bars 1-4 can be varied using the following ranges:

Bar 1: Evaporative yarn with Denier range—10 Denier-200 Denier, Filament range—1 filament-400 filaments

Bar 2: Absorbent yarn with Denier range—10 Denier-200 Denier, Filament range—1 filament-400 filaments

Bar 3: Evaporative yarn with Denier range—10 Denier-200 Denier, Filament range—1 filament-400 filaments

Bar 4: Elastomeric yarn with Denier range—10 Denier-340 Denier

As another example, Bar 2 may utilize a yarn such as Nanofront polyester yarn manufactured by Teijin which has significantly smaller filaments than traditional absorbent yarns.

Another embodiment of cooling fabric 100 uses the following 4-bar knitting stitch and yarn combination:

Bar 1-1-0/2-3 (evaporative yarn such as ASKIN)

Bar 2-1-2/1-0 (absorbent yarn such as MIPAN XF)

Bar 3-0-1/2-1 (evaporative yarn such as ASKIN)

Bar 4-1-0/1-2 (elastic yarn such as Spandex).

In this stitch configuration, bar 1 is a 45 Denier/24 filament polyester fully drawn yarn; bar 2 is a 50 Denier/48 filament polyester and nylon conjugated fully drawn yarn; bar 3 is a 75 Denier/36 filament polyester draw textured yarn; and bar 4 is a 40 Denier spandex.

In both knitting stitch examples, bars 1 and 3 are cool touch/quick dry/absorption materials as have already been described. The Qmax for these yarns is greater than 0.140 W/cm<sup>2</sup> on the face side and 0.120 W/cm<sup>2</sup> on the back side of the material which indicates a cooling touch effect as has already been described. The wet Qmax for these yarns is greater than 0.280 W/cm<sup>2</sup> on face side and 0.180 W/cm<sup>2</sup> on back side. Bar 2 is a conjugated highly absorbent yarn (MIPAN XF) which has a wicking rate and a wicking distance more than twice that of cotton of equivalent density. The spandex yarn provides hydrophobic properties, provides stretch properties, and a draping effect.

Additional Performance Yarn

An embodiment of the present invention is the use of other performance yarns to enhance evaporative and absorbency effects. Specifically, for the yarns listed in layers 104 and 108, other evaporative yarns with additional performance properties can be added, blended, or twisted with the evaporative yarns to intensify the cooling effect of fabric 100. Possible additional evaporative yarns include, but are not limited to, the following:

Mineral containing—An embodiment of the present invention involves incorporating yarns impregnated with various minerals such as mica, jade, coconut shell, volcanic ash, etc. These mineral containing yarns could be added to first layer **104** or third layer **108** to provide a cool touch and/or increased evaporative performance. Mineral yarn could be used to also provide greater surface area for added evaporation power. An example of this type of mineral containing yarn is 37.5 polyester or 37.5 nylon, both of which are manufactured by Cocona, Inc. Both of these example yarns contain particles permanently embedded at the fiber level which capture and release moisture vapor. The active particles provide approximately 800% more surface area to the fiber and also provide a unique driving force to remove moisture vapor. By actively responding to body heat, the active particles use this energy from the body to accelerate the vapor movement and speed up the conversion of liquid to vapor, significantly increasing drying rates. Using highly evaporative yarns allows for increase evaporation from the absorbent layers.

Absorbent yarns—An embodiment of the present invention includes the use of highly absorbent yarns such as bi-component synthetic, alternative modified cross-section synthetic yarn, cellulosic, and non-cellulosic blended yarns. This can include both filament and spun yarn and yarn combinations thereof which can be incorporated into layer **106**. This also includes yarns described in U.S. Pat. No. 9,506,187 entitled “Textile Dyeing Using Nanocellulosic Fibers.” Other absorbent yarns may include Nanofront polyester yarn manufactured by Teijin. For example, some Nanofront polyester filaments have a diameter of 400 nanometers, or 22500, times smaller than the cross-sectional area of a strand of hair.

Phase Change—Phase change yarns such as “Outlast” polyester and “Outlast” nylon, both of which are manufactured by Outlast Technologies LLC, can be incorporated into layer **106**. Other cellulosic and non-cellulosic blended fibers as described above can be added to layer **106** the present invention to provide added cooling power and cooling touch.

#### Finishing Practices

In addition to normal textile finishing practices, an embodiment of the present invention includes applying extra finishing practices before or after construction of cooling fabric **100** which impart added cooling power, duration, temperatures and other cooling performance properties when the cooling fabric **100** is wetted to activate. The following provides examples of additional finishing practices suitable for use with cooling fabric **100**. Combinations of the following methods may also be employed.

Burn out—Using a combination of yarns allows certain yarns to be chemically burned out of the material. This allows certain portions of the material to maintain a complete bundle of cooling yarns while other burned-out sections will not contain the complete bundle of cooling evaporative and absorbent yarns. This finishing method therefore allows for higher air transfer between burned out and non burned out sections, thereby adding to the evaporation rate and increased cooling ability. The burn-out finishing technique also allows for a mapping or patterns for areas of higher and lower cooling ability to be designed for a specific end-use. As an example, a yoga cooling towel will have a different burn out engineered burned-out patterning than a cooling shirt designed as a base layer under football pads.

Brushing and Shearing—Brushing, using methods such as pin brushing or less obtrusive ceramic paper brushing, provides pile height to the cooling fabric. This pile height provides a softer hand feel aesthetically and added absorbent ability. Additionally, added surface area for water evaporation helps speed the rate of evaporation. In addition to the pin brushing method, shearing the fabric surface to a select pile height or variable pile heights can create differential evaporation rates within the same textile. A diagram of a pin-type brushing machine is depicted in FIG. 4. As shown, one face of the cooling fabric **100** is fed over pin brusher **402** which rotates in a direction opposite to the direction that fabric **100** is fed. As cooling fabric **100** passes over pins **404**, the pins slowly brush the surface of cooling fabric **100**, leaving the back unscathed. In some embodiments, both sides of cooling fabric **100** can be brushed.

Embossing—Embossing creates a reorientation of the fibers on the fabric surface. This finishing method is used to add surface area by flattening the yarn surface. This added surface area allows for a higher evaporation rate which thereby creates additional cooling properties and a higher level of evaporation. A diagram of an embossing machine and process is depicted in FIG. 5. Here, the cooling fabric **100** is fed between heated roller **502** and non-heated roller **504**. The surface of heated roller **502** generally contains the pattern which is to appear on the final embossed fabric. In other embodiments, the fabric may be reversed if both sides of cooling fabric **100** are to be embossed.

Brushed+Embossed—Using a combination of brushing and embossing can impart added cooling properties to the cooling fabric. Brushing and Embossed performance benefits are both described above. A sample of textured cooling fabric **100** is depicted in FIG. 6 which has been both brushed and embossed.

#### Fabric Construction & Yarn Positions

A variety or combination of any of the following described constructions can impart added cooling power, duration, and lower temperatures when the cooling fabric is wetted to activate.

Yarn placement/position changes—The conjugate yarn used in layer **106** can also be used in other layers such as layer **104** (e.g., combined on bar 1, FIG. 3A) and combined with the evaporative yarn and spandex. This added yarn would provide more absorption power against the skin **102**.

Warp knit pattern changes—The warp knit patterns described with respect to FIGS. 3A-3E can be modified while still producing a similar layering effect depicted in FIG. 1. For example, in FIG. 3A, bar 1-0/2-3 can be modified to 1/0-3/4.

Warp Knit Spacer—A similar layering effect depicted in FIG. 1 can also be achieved using a warp knit spacer. A warp knit spacer machine has the added capability of inserting additional yarns such as a mono-filament yarn to provide added thickness to the cooling fabric **100**. This added thickness created by yarns such as mono-filament yarns can be substituted or combined intermittently with conjugate yarn while the outside yarns used can be highly evaporative yarns or previously described yarns.

Warp Knit Jacquard—A similar layering effect depicted in FIG. 1 can also be achieved using a warp knit jacquard. A warp knit jacquard can be utilized to create unique patterns such as but not limited to lace, fancy knits,

mesh, body mapped, and other three-dimensional designs. Warp knit jacquard can creatively place highly evaporative yarns with highly absorbent yarns within the same construction to create a uniquely designed cooling fabric with or without patterns such as mesh and graphics.

**Circular Knit Spacer**—A similar layering effect depicted in FIG. 1 can also be achieved using a circular knit spacer. A circular knit spacer machine has the added capability of inserting additional yarns such as a monofilament yarn to provide added thickness to the material. This added thickness created by yarns such as monofilament yarn can be substituted or combined intermittently with conjugate yarn while the outside yarns used can be highly evaporative yarns or any previously described yarns.

**Circular Knit Interlock, Ponte', Pique**—A similar layering effect depicted in FIG. 1 can also be achieved using a circular knit interlock, ponte, or pique constructions. A circular knit interlock machine has the added capability of inserting additional evaporative and absorbent yarns to provide added evaporative cooling ability to the fabric.

**Circular Knit Jacquard**—A similar layering effect depicted in FIG. 1 can also be achieved using a circular knit jacquard. A circular knit jacquard can be utilized to create unique patterns, such as, but not limited to, fancy knits, mesh, body-mapped patterns, and other three-dimensional designs. Circular knit jacquard can creatively place highly evaporative yarns with highly absorbent yarns within the same construction to create a uniquely designed cooling fabric with or without patterns such as mesh and graphics.

**Flat bed knitting**—A similar layering effect depicted in FIG. 1 can also be achieved using a flat knitting machine. A flat knitting machine is very flexible, allowing complex stitch designs, shaped knitting and precise width adjustment. The two largest manufacturers of industrial flat knitting machines are Stoll of Germany, and Shima Seiki of Japan.

**Seamless and Hosiery Construction and Yarns**  
Seamless constructions require the use of a single yarn feed (which is typically a combination of nylon or polyester plus spandex) during construction. This single feed can be a single yarn or composed of multiple yarns during construction. In a first described embodiment, described is a multi-filament yarn construction that can be used in seamless constructions (e.g., for hosiery) that provides the same cooling effect as cooling fabric 100 described with reference to FIGS. 1-9. FIG. 7A illustrates a first yarn construction 700 compatible with seamless constructions. As shown, the core 702 of the yarn 700 is composed of multiple filaments of a stretchable yarn such as Lycra or spandex at various deniers. Additionally, the core 702 preferably comprises multiple filaments of a highly absorbent yarn such as that used in layer 106 of cooling fabric 100. Preferably, the absorbent yarn is a conjugated bi-component polyester and nylon yarn with having filaments with a special star-shaped cross-section as depicted in FIG. 3B.

The core 702 is either double covered (FIG. 7A), single-covered (FIG. 7B), air jet covered (FIG. 7C), or corespun (FIG. 7D) by multiple filaments of evaporative yarn 704 such as that used in first layer 104. The evaporative yarn of covering 704 is preferably a nylon or polyester yarn having filaments with a unique cross-section (as seen in FIG. 2A) and is embedded with minerals (e.g., jade or mica) to

transport and evaporate moisture from skin 102 to core 700 while still providing a cooling touch.

When yarn 700 is used in a seamless construction, the evaporative yarn, located in covering 704, rests against the skin of the user and it wicks moisture to the core 700. The moisture can then leave the fabric through covering 704 which is also exposed to the air (i.e., because it surrounds the core 700 on all sides). In this way, yarn 700 can be used to provide a similar layering effect to that of cooling fabric 100 depicted in FIG. 1.

An example of a seamless knit construction utilizing yarn 700 is depicted in FIG. 8. FIG. 9A depicts a front face of a seamless knit fabric utilizing yarn 700 and FIG. 9B depicts a rear face of the same seamless knit fabric. As can be seen, the front and rear faces of the seamless knit fabric have different patterning. With seamless, patterns are easily altered and practically an unlimited amount of patterns are available.

Other methods can also be used to form yarn 700 as depicted in FIGS. 7C and 7D. The yarn 700 depicted in FIG. 7C employs an air jet covering technique to cover core 702 (stretchable and absorbent yarns) with covering 704 (evaporative yarns). And, as depicted in FIG. 7D, the stretchable and absorbent yarns, are wrapped with evaporative yarns and core-spun into a single yarn 700 which can also be used in seamless knit constructions.

Seamless knit constructions have the advantage of being tubular and can be used to create unique patterns to impart added or lessened cooling zones within the material. The yarns shown in FIGS. 7A-7D can also be used to create woven fabrics.

In other embodiments, the yarn used in the seamless or hosiery construction can be a single feed utilizing any combination of the yarns containing the filaments shown in FIGS. 2A-2D. For example, a first yarn used in the feed may be a combination of a highly absorbent yarn with a evaporative yarn and a second yarn may be a multiple filament spandex yarn. In practical terms, the highly absorbent yarn can be plated separately into any seamless construction which also contains evaporative yarns to create a cooling material.

The present invention has been described with respect to various examples. Nevertheless, it is to be understood that various modifications may be made without departing from the spirit and scope of the invention as described by the following claims.

The invention claimed is:

1. A multi-layered knitted cooling fabric comprising:  
a first layer formed by a first yarn,  
wherein the first yarn is an evaporative yarn;  
a second layer adjacent the first layer formed by a second  
yarn,  
wherein the second yarn is an absorbent yarn having an  
absorbency at least twice that of cotton of equivalent  
density;  
a third layer adjacent the second layer formed by a third  
yarn,  
wherein the third yarn is an evaporative yarn config-  
ured to allow moisture trapped in the second layer to  
move into the third layer.

2. The multi-layered knit cooling fabric of claim 1,  
wherein the multi-layered knit cooling fabric cools to up to  
30° F. below an average body temperature of approximately  
98.6° F. when wetted and activated.

3. The multi-layered knit cooling fabric of claim 1,  
wherein the multi-layered knit cooling fabric is constructed

using a warp knit stitch selected from the stitch group consisting of tricot, raschel, spacer, and lace.

4. The multi-layered knit cooling fabric of claim 1, wherein the multi-layered knit cooling fabric is constructed using a knitting construction selected from the group consisting of a warp knit spacer construction, a warp knit jacquard construction, a circular knit spacer construction, a circular knit jacquard construction, a flat bed knitting construction, and a circular knit interlock, pique, ponte construction.

5. The multi-layered knit cooling fabric of claim 1, wherein the first yarn is an evaporative and UV-protective yarn.

6. The multi-layered knit cooling fabric of claim 1, wherein the second yarn is a conjugated bi-component polyester and nylon yarn.

7. The multi-layered knit cooling fabric of claim 1, where the second yarn has a wicking rate and a wicking distance more than twice that of cotton of equivalent density.

8. The multi-layered knit cooling fabric of claim 1, wherein the third yarn is an evaporative and UV-protective yarn.

9. The multi-layered knit cooling fabric of claim 1, wherein the multi-layered knit cooling fabric has a density of 100-600 g/m<sup>2</sup>.

10. The multi-layered knit cooling fabric of claim 1, wherein the first layer additionally comprises spandex.

11. The multi-layered knit cooling fabric of claim 1, wherein the first yarn is a conjugated bi-component polyester and nylon yarn with a special star-shaped cross-section.

12. The multi-layered knit cooling fabric of claim 1, wherein the fabric forms an entire garment.

13. The multi-layered knit cooling fabric of claim 1, wherein the garment includes a shirt, pants, and/or shorts.

14. The multi-layered knit cooling fabric of claim 1, wherein the fabric is integrated into a garment.

15. The multi-layered knit cooling fabric of claim 1, wherein the fabric forms a headband, a towel, and/or a hat.

16. The multi-layered knit cooling fabric of claim 1, wherein the first layer is adapted to be worn against skin.

17. The multi-layered knit cooling fabric of claim 1, wherein the first layer includes a combination of a stretchable synthetic yarn and the evaporative yarn.

18. The multi-layered knit cooling fabric of claim 1, wherein the third layer is adapted to be exposed to an external environment.

19. The multi-layered knit cooling fabric of claim 1, wherein the second layer is arranged between the first layer and the third layer.

20. The multi-layered knit cooling fabric of claim 1, wherein the first layer includes hydrophobic and hydrophilic channels.

\* \* \* \* \*